

W. E. GREENAWALT.  
PROCESS OF TREATING MATERIALS ELECTROLYTICALLY.  
APPLICATION FILED MAY 13, 1913.

1,209,835.

Patented Dec. 26, 1916.



FIG 1



FIG 2

WITNESSES:

*Jesse G. Lefler*  
*Fred L. Scott.*

INVENTOR.

*William E. Greenawalt*

# UNITED STATES PATENT OFFICE.

WILLIAM E. GREENAWALT, OF DENVER, COLORADO.

## PROCESS OF TREATING MATERIALS ELECTROLYTICALLY.

1,209,835.

Specification of Letters Patent. Patented Dec. 26, 1916.

Application filed May 13, 1913. Serial No. 767,392.

To all whom it may concern:

Be it known that I, WILLIAM E. GREENAWALT, a citizen of the United States, residing in the city and county of Denver and State of Colorado, have invented certain new and useful Improvements in Processes of Treating Materials Electrolytically, of which the following is a specification.

It makes it possible to treat successfully such substances as copper matte, copper sulfid precipitate, cement copper, zinc oxid, copper oxid, lead sulfate, lead sulfid, metallic lead, etc. It also finds application in the electrolysis of solutions with insoluble anodes, where the disintegrated anode material has hitherto been a source of annoyance and expense.

In the treatment of substances such as copper matte or copper sulfid precipitate, the liberated sulfid ordinarily adheres to the anode and thus increases the electrical resistance to such an extent as to make the process unworkable. In the electrolysis of copper matte, as for example in the Marchese process, the deposited copper was exceedingly impure and contained all impurities originally in the matte. By my process these difficulties are easily overcome.

In the refining of cement copper the customer is to smelt it to blister copper and then refine it electrolytically. Such a method can only be carried out on a large scale and is too expensive to be profitably worked in copper mining districts, and hence producers of cement copper are obliged to market their product to the refineries or smelting companies, to their disadvantage. By my process the cement copper is at once refined, without fusion, and the precious metals obtained separately. Similarly, in the electrolysis of lead used as anode in sulfate solutions; the lead is peroxidized and forms a coating which increases the electrical resistance to a prohibitive degree, and its accumulation in the electrolyzer ultimately leads to short circuiting of the current and other disturbances, so that it has to be removed at frequent intervals at considerable expense, and hence lead anodes offer disadvantages so great as to be of little use. In this process these difficulties are overcome; the peroxid of lead forms to a less degree and that which is formed is at once removed from the anode and from the electrolyzer, and consequently

from the sphere of disturbance of the electric current.

This process also presents ideal conditions for the electrolysis of salts, such as copper oxid, zinc oxid, lead sulfate or sulfid, and so that the operation can be continuously and cheaply carried on.

Referring to the accompanying drawings, Figure 1 represents a suitable apparatus for carrying out the process, and Fig. 2 a modification.

In the figures 1 represents an electrolyzer having one electrode 2, at the bottom and the opposite electrode 3, suspended over it. Separating the two electrodes is a diaphragm 4, attached preferably to an electrode bell or frame 5, thereby forming a separate compartment. The diaphragm and bell or frame are supported by suspenders 6, which are arranged so that the frame, or bell, may be adjusted vertically, while being oscillated horizontally from pivotal points 21 by the mechanism 7.

8 represents a flexible duct to permit the circulation of the electrolyte through the electrode bell while it is being oscillated, and flows into tank 10, from whence, by means of pump 11 and pipe 12, it may be returned to the electrode bell. Similarly, the solution may be circulated through the electrolyte tank by means of the pipe 13, to the tank 14, and returned to the electrolyte tank by means of the pump 15 and the pipe 16.

Having now given a description of the preferred apparatus, the process will be described, first, in the treatment of copper sulfid using the apparatus as shown in Fig. 1, and second, using the apparatus as shown in Fig. 2.

Referring now more particularly to Fig. 1, the copper sulfid 20, which may be fused or unfused, granulated or in slabs, is placed on the insoluble lead anode sheet in the bottom of the tank, in an electrolyte of copper sulfate and sulfuric acid. The current is turned on and the cathode bell 5 oscillated by the mechanism 7. The first effect of the oscillation is to make a muddy solution in the tank due to the agitation of the anolyte which brings the finer particles of copper sulfid and liberated sulfur in suspension. If it were not for the diaphragm the matter in suspension would get to the cathode and contaminate the deposit. The effect of the elec-

trolysis is to decompose the copper sulfid, the copper being deposited on the cathode 3, and the sulfur liberated on the surface of the copper sulfid. The sulfur, being lighter than the copper sulfid, is readily brought into suspension in the anolyte due to the oscillation of the diaphragm and supporting frame, and by circulating the anolyte through pipe 13 to tank 14, where the sulfur is settled out, the clear solution may be pumped back to the electrolyte tank by means of pump 15 and pipe 16. Similarly the electrolyte may be circulated through the cathode compartment, especially if the deposit is spongy and does not adhere to the cathode. If the deposit is spongy or granular it is detached from the cathode by the oscillating diaphragm and held in suspension until expelled from the electrolyzer, and flows into tank 10 where the copper settles out and the clear solution pumped back to the cathode bell through pump 11 and pipe 12. If the deposit on the cathode is firm, as it will be if a low current density is used, the deposit is stripped from time to time, and the cathodes returned to the electrolyzer. In this way, it will be seen, that the work can progress continuously, the copper being deposited and the sulfur liberated and removed from the cell so that no deleterious results follow its liberation. The gold, silver, and lead, and perhaps other metals, will be found in the anode sludge and may be removed as such, or with the sulfur, in suspension. If removed with the sulfur, they may be recovered when the sulfur is refined. The cross pieces on the anode bell supporting the diaphragm, are effective in agitating the electrolyte in both the anode and cathode compartments, and thus are largely instrumental in promoting the process. These cross pieces may be transverse or longitudinal; the transverse arrangement is preferred. Deleterious gases from the under side of the diaphragm escape through the holes or saw cuts 22.

Suppose, now, that copper sulfid is to be electrolyzed in the modified apparatus, as shown in Fig. 2. As a preliminary step it is best to cast the sulfid into anodes, 3, and suspend them in the anode bell 5, and then make suitable electrical connections. A sheet copper cathode 2, is placed in the bottom of the electrolyte tank 1, to receive the copper deposit. When the current is turned on and the diaphragm oscillated, copper will be deposited on the cathode and sulfur released at the anode, which owing to the oscillating diaphragm and consequent agitation of the electrolyte on the face of the anode, drops off, but is held in suspension in the electrolyte, and is withdrawn with the electrolyte through pipe 9, into the settling tank, where the sulfur is separated from the electrolyte and the electrolyte returned to

the electrolyzer. In this way the circulation is continued indefinitely, copper being deposited, and the sulfur continuously and automatically removed by means of the oscillating diaphragm.

70

If a depolarizing agent, such as sulfur dioxide, is to be introduced into the electrolyte, it is best brought into solution in the settling tanks 10 and 14. Similarly, any substance capable of promoting the process, may be introduced in the electrolyte as it is circulated to effect the separation of the material in suspension, derived from the electrolysis.

75

If cement copper is to be refined, it is placed on the lead anode 2, in the bottom of the tank and shown in Fig. 1 by 20, and the operation conducted as for copper sulfid. The precious metals and other valuable constituents may be subsequently recovered from the residual slimes.

85

If lead is used as the anode, in the electrolysis of solutions, such as copper sulfate, the peroxid formed from the lead anode 3, Fig. 1, is removed from the anode and from the electrolyzer by the circulating electrolyte, due to the oscillation of the diaphragm.

90

By the introduction of the oscillating diaphragm, as proposed in my process, the following distinctive results are attained: First; simultaneous agitation of both the anolyte and catholyte. Second; freeing of the insoluble disintegrated electrode material from the electrode and maintaining it in suspension in the electrolyte. Third; removing of the disintegrated electrode material from the electrolyzer and from the sphere of action of the electric current. Fourth; preventing of the suspended matter from getting to the deposited metal. Fifth; if the diaphragm oscillates between stationary electrodes the expense of oscillation or moving the heavy electrode material is entirely obviated. Sixth; removal of air and other gases from the diaphragm and from the electrodes, and thus preventing polarization, and the loss of efficiency due to impoverishment of the electrolyte in contact with the electrodes. Seventh; the electrode plate in the bottom of the tank, which receives the material to be treated, is an effective way of making electrical contact between a loose material and the conductor.

95

The process also finds application in the direct refining of gold and silver precipitate as obtained either by the chlorination, cyanid, or hyposulfite processes. It may also be employed to continuously remove spongy deposits from the cathode, and this action may go on simultaneously with the removal of the disintegrated or insoluble anode material. The loosening of the disintegrated material, such as lead peroxid, is facilitated by the introduction of a reagent, such as sulfur dioxide, and may be further facil-

100

105

110

115

120

125

130

tated by using an alternating current in connection with the direct current. If a depolarizer is used, the acid in the electrolyte is increased, and in this way its amount 5 may be regulated.

The process also finds application in the electrolysis of lixivants, such as cyanid in the treatment of gold and silver ores, whereby the metals may be deposited into a mercury cathode in the bottom of the electrolyzer, and recovered as amalgam, from 10 which the metals may be subsequently obtained by the distillation of the mercury.

If a material is electrolyzed in which the 15 diaphragm may be dispensed with, the diaphragm may be omitted and the frame attached to the anode bell used as an agitator.

If the material to be electrolyzed is in a 20 finely divided condition, either compartment may be regarded as the anode compartment, and either compartment may be regarded as the cathode compartment.

I claim:

1. An electrolytic process which consists in 25 maintaining separate the anolyte and catholyte with a suitable diaphragm, simultaneously agitating both the anolyte and catholyte and withdrawing the electrolyte from one compartment and passing it through the other compartment without mingling with the electrolyte of the other compartment.

2. A process which consists in electrolyzing 30 metallic salts in a finely divided condition which consists in simultaneously agitating both the anolyte and catholyte while maintaining separate the anolyte from the

catholyte, and while maintaining a relative motion between the electrodes and the metallic salts being electrolyzed. 40

3. A process which consists in electrolyzing finely divided material in which the anolyte is separated by a diaphragm from the catholyte, and agitating the material to keep it in suspension during electrolysis, and 45 maintaining a relative motion between the electrodes and the finely divided material being electrolyzed.

4. A process which consists in electrolyzing finely divided material and agitating the 50 material to keep it in suspension in the electrolyte during electrolysis while maintaining the anolyte separate from the catholyte, and withdrawing the electrolyte from one compartment and passing it through the other 55 compartment without mingling with the electrolyte in the other compartment.

5. An electrolytic process which consists in maintaining separate the anolyte from the catholyte with a suitable diaphragm, 60 simultaneously agitating both the anolyte and catholyte, subjecting the material being treated to the action of electrolysis with a direct current with insoluble anodes thus causing a disintegration of the anode material, and facilitating the loosening of the disintegrated anode material by the action 65 of an alternating current working in connection with the direct current.

WILLIAM E. GREENAWALT.

Witnesses:

FRED L. SCOTT,  
JESSIE G. SELLERS.